

## UNITED STATES PATENT OFFICE.

WILLIAM N. BLAKEMAN, JR., OF NEW YORK, N. Y.

## PAINT COMPOUND OR MIXTURE.

SPECIFICATION forming part of Letters Patent No. 767,683, dated August 16, 1904.

Application filed August 11, 1903. Serial No. 169,096. (No specimens.)

*To all whom it may concern:*

Be it known that I, WILLIAM N. BLAKEMAN, Jr., of the borough of Manhattan, in the city, county, and State of New York, have invented 5 a new and useful Paint Compound or Mixture, which invention is fully set forth in the following specification.

The object of this invention is to utilize non-drying fatty oils (such as cotton-oil, sunflower-oil, corn-oil, castor-oil, and the like) in the manufacture of paints, these oils having heretofore been regarded as useless for this purpose by reason of their non-drying characteristic.

15 My invention consists in incorporating with a non-drying oil a small proportion of tung-oil, (known also as "Chinese" or "Japanese" wood-oil) and then grinding a pigment in this vehicle.

20 Tung-oil seems to be a very remarkable oleaginous product, the composition of which is not now well understood, and although classed among the drying-oils the result of its induration is very different from the oxidized film of 25 the well-known drying-oils, for when exposed to the atmosphere in a thin layer on plain surfaces it dries to a rough, opaque, and arborescent film.

I have discovered that when about fifteen 30 per cent. of tung-oil is incorporated with one of the non-drying fatty oils—cotton-oil, for example—the compound or mixture will form a drying-oil possessing good drying qualities and well adapted for use as a vehicle for pigments for paints.

In carrying out my process I simply take the desired proportions of each oil and thoroughly incorporate one with the other. Either the tung-oil or the non-drying fatty oil, or 40 both, may be oxidized before being combined and a more energetic and complete blending thereby effected. The tung-oil may be combined with a mixture of two or more non-drying oils, and from five to ten per cent. of linseed or other drying oil (either raw or boiled) 45 may be added as a drier, if desired, in which case the proportion of tung-oil may be slightly reduced. In order to form a paint compound, I then grind in the oil vehicle so produced any 50 of the well-known pigments, such as white lead, lead sulfate, lead sulfite, zinc oxid, zinc oxychlorid, zinc sulfid, zinc oxysulfid, zinc

sulfo-chlorid, or barium sulfate, or any combination of these. I prefer to use either lead sulfate, zinc oxid, zinc sulfid, zinc oxychlorid, 55 or zinc sulfo-chlorid. The paint compound so produced will when spread dry in a satisfactory manner and with a smooth and elastic film. Even white lead and other lead salts (which heretofore it has been found impossible to use with the non-drying fatty oils) will 60 form quick-drying compounds with non-drying oils treated as herein described.

The proportions of oils and pigments may be varied as practice shall dictate. The proportion of tung-oil which I use is from about ten per cent. as a minimum to twenty-five per cent. as a maximum, depending upon the nature of the non-drying oil and character of the pigment used, fifteen per cent. giving satisfactory results in nearly every case. If zinc 70 oxid be used as a pigment, suitable proportions would be eighty-five parts of cotton-oil, fifteen parts of tung-oil, and one hundred parts of zinc oxid.

In another application, Serial No. 169,095, filed herewith, I have claimed a drying-oil composed of tung-oil and a non-drying fatty oil; but in the present application I desire to claim 75 said oil in combination with a pigment.

Having thus fully described my invention, I claim—

1. As a new composition of matter, a paint compound or mixture of, substantially, eighty-five parts of non-drying fatty oil, fifteen parts 85 of tung-oil, and a pigment.

2. As a new composition of matter, a paint compound or mixture of, substantially, eighty-five parts of cotton-oil, fifteen parts of tung-oil, and a pigment.

3. As a new composition of matter, a paint compound of tung-oil; an oxidized non-drying fatty oil; and a pigment.

4. As a new composition of matter, a paint compound of oxidized tung-oil, an oxidized 95 non-drying fatty oil, and a pigment.

5. As a new composition of matter, a paint compound or mixture of, substantially, eighty-five parts of non-drying fatty oil; fifteen parts of tung-oil; a pigment; and a drier.

WM. N. BLAKEMAN, JR.

Witnesses:

FRANCIS P. REILLY,  
CHAS. A. KANE.